

Jan. 15, 1963

J. COHEN ET AL

3,073,731

PLASTICIZING AGENTS FOR NITROCELLULOSE

Filed March 29, 1956

2 Sheets-Sheet 1



INVENTORS  
RONALD A. HENRY  
WILLIAM G. FINNEGAN  
JOSEPH COHEN

BY *J. A. O'Brien*

*K. F. Ross*

ATTORNEYS

Jan. 15, 1963

J. COHEN ET AL

3,073,731

PLASTICIZING AGENTS FOR NITROCELLULOSE

Filed March 29, 1956

2 Sheets-Sheet 2

*Fig. 3.*



*Fig. 4.*



INVENTORS  
RONALD A. HENRY  
WILLIAM G. FINNEGAN  
JOSEPH COHEN  
BY  
*J. D. O'Brien*  
*H. F. Ross*  
ATTORNEYS

1

3,073,731

PLASTICIZING AGENTS FOR NITROCELLULOSE  
 Joseph Cohen, Arcadia, and William G. Finnegan and  
 Ronald A. Henry, China Lake, Calif., assignors to the  
 United States of America as represented by the Secre-  
 tary of the Navy

Filed Mar. 29, 1956, Ser. No. 574,939

11 Claims. (Cl. 149—92)

(Granted under Title 35, U.S. Code (1952), sec. 266)

The invention described herein may be manufactured and used by or for the Government of the United States of America for governmental purposes without the payment of any royalties thereon or therefor.

This invention relates to improved propellant compositions for jet actuated devices, more particularly, it relates to propellant compositions incorporating improved plasticizers.

In the art of compounding propellant compositions for jet actuated devices it is well known that plasticizers are essential to the compositions for providing the required plasticity to permit homogeneous mixing of the raw materials and to provide a finished propellant grain which is well plasticized and not subject to cracking or breaking. A suitable plasticizer, in addition to being capable of imparting plasticity to the propellant composition and to the finished propellant grain, must possess a number of other well defined properties. Its presence in the composition should not undesirably affect the highly sensitive ballistic properties of the propellant, such as, the mesa and plateau effect of propellants for jet actuated devices. Further, incorporation of the plasticizer in the propellant composition should not undesirably affect the surveillance characteristics and thermochemical properties of the composition. Additionally, the plasticizing agent should preferably have a high nitrogen content, thus assuring a low average molecular weight for the combustion products.

Representative plasticizers ordinarily incorporated in double base propellant powders are dialkyl phthalates such as dimethyl and diethyl phthalate, ethyl centralite, dibutyl sebacate and nitroglycerin, the latter being an explosive plasticizer. None of these plasticizers, with the exception of ethyl centralite, function to remove certain oxides of nitrogen generated in propellants during storage which shorten the storage life of the propellants. Further, of the named compounds only nitroglycerin contains an appreciable percentage of nitrogen.

It is, therefore, an object of this invention to provide propellant compositions for jet actuated devices possessing a high degree of plasticization.

It is another object of this invention to provide highly plasticized propellant compositions for jet actuated devices which have good ballistic and thermochemical properties as well as good surveillance properties.

It is still another object of this invention to provide homogeneous propellant formulations in which the plasticizer, in addition to its plasticizing effect, also functions as a coolant by providing a large percentage of nitrogen.

It is a further object of this invention to provide propellant compositions for jet actuated devices which produce combustion products having a low average molecular weight.

It has been found that the above and other objects are accomplished by homogeneously incorporating derivatives of tetrazole into propellant compositions in amounts varying from about 5 percent to about 50 percent, depending upon the particular derivative and the compositions into which it is incorporated.

The derivatives of tetrazole disclosed herein as plasticizers have a high nitrogen content, generally over 30 percent, the parent compound itself having a nitrogen

2

content of 80 percent. This is contrasted with the 10.4 percent of nitrogen in ethyl centralite and 18.5 percent of nitrogen in nitroglycerin. Further some of these derivatives have the property of absorbing oxides of nitrogen released from propellants on standing. An advantage of the derivatives of tetrazole over prior non-explosive plasticizers for propellant compositions for jet actuated devices is the superior degree of gelation or colloidalizing of nitrocellulose produced by them. When they are mixed with nitrocellulose they produce a gel of varying degree, dependent upon the particular derivative which is used and on the relative percentages of the derivative and the nitrocellulose. When a complete propellant composition is processed to contain nitrocellulose, the tetrazole derivative, nitroglycerin, and the various other conventional additives to propellants for jet actuated devices, such as ballistic modifiers, stabilizers, and others, the colloidalizing effect on the nitrocellulose is so effective that a uniformly distributed matrix incorporating the other ingredients of the composition is formed. Furthermore, the absorption by nitrocellulose of other ingredients of the composition which are ordinarily physically compatible with nitrocellulose, is not inhibited by the presence of the tetrazole derivatives. Illustrative of the superior plasticizing effect of the tetrazole derivatives is the fact that, whereas it is common practice to include approximately equal weights of nitrocellulose and total plasticizer in double base propellant compositions it has been found that the ratio of nitrocellulose to the total amount of plasticizer, when one of the tetrazole derivatives is included, can be as high as 2 to 1 and still give a properly colloided composition. This is illustrated by a comparison of the plasticizing effects produced in a conventional propellant composition by a standard plasticizer, ethyl centralite, and by a representative member of the tetrazole derivatives, 1-ethyl-5-ethylaminotetrazole, the compositions being as follows:

|                                             | I (weight percent) | II (weight percent) |
|---------------------------------------------|--------------------|---------------------|
| Nitrocellulose (12.6% N).....               | 19.1               | 29.84               |
| Nitroglycerin.....                          | 18.6               | 7.86                |
| Nitroguanidine.....                         | 54.8               | 54.8                |
| Ethyl centralite.....                       | 7.5                | 0.0                 |
| 1-ethyl-5-ethylaminotetrazole.....          | 0.0                | 7.5                 |
| Ratio of nitrocellulose to plasticizer..... | 0.73 to 1.0        | 1.94 to 1.0         |

Despite the substantially larger ratio of total plasticizer to nitrocellulose in the composition of Example I, strands produced from the composition of Example II were found to be less brittle and more flexible than those produced from the composition of Example I.

The invention is best understood by reference to the description which follows, taken in connection with the drawings, which form a part of this specification and in which the FIGS. 1-4, inclusive, are graphs of the pressure-burning rate relationship of propellant compositions of the invention.

Table I below contains 24 examples of propellant compositions of the invention which were selected as representative from among those prepared and tested. The examples include a sampling of compositions containing 13 representative tetrazoles as plasticizers, some tetrazoles being used in more than one composition. Examples 1-7, inclusive, 9-13, inclusive, and 15-20, inclusive, and 24 are examples of propellants made by incorporating the tetrazole plasticizers in conventional double base propellants, the propellant composition being set forth in the table. Examples 22, 23, 25, 26 and 27 are of propellant compositions made by incorporating tetrazole plasticizers in cool gun propellant formulations. Examples 8 and 14 are blanks using conventional double base components,

which were made for comparative purposes. Example 21 is a blank of a conventional cool gun propellant composition, cordite-N. All of the formulations were made by the solvent process, a conventional manufacturing method used for double base and cool gun propellants. Other processes may be used, the only requirement being that a process be used which insures that the plasticizer is uniformly and homogeneously incorporated throughout the propellant in its finished state. This can only be insured by a thorough mixing and incorporating of the plasticizer in the form of small particles in the raw propellant mix, such as is done in the solvent or solventless process mentioned above.

The following compounds were tested as plasticizers with nitrocellulose and found to be compatible and excellent plasticizers at the percentage level indicated.

| Compound                                                 | Percent compound |
|----------------------------------------------------------|------------------|
| Ethyl (1-methyl-5-tetrazolyl)acetate                     | 20               |
| Ethyl (2-methyl-5-tetrazolyl)acetate                     | 40               |
| $\beta$ -(1-tetrazolyl)ethyl acetate                     | 40               |
| $\beta$ -(2-tetrazolyl)ethyl acetate                     | 40               |
| Ethyl (2-tetrazolyl)acetate                              | 20               |
| Mixture of 1,4-bis (1 and 2-methyl-5-tetrazolyl) butanes | 20               |

TABLE I

[Weight percent]

| Example                                | 1  | 2  | 3   | 4    | 5   | 6   | 7  | 8     | 9     | 10   | 11   | 12    | 13    | 14    | 15    | 16   | 17 | 18   | 19    | 20    | 21   | 22    | 23    | 24    | 25    | 26    | 27    |   |
|----------------------------------------|----|----|-----|------|-----|-----|----|-------|-------|------|------|-------|-------|-------|-------|------|----|------|-------|-------|------|-------|-------|-------|-------|-------|-------|---|
| INGREDIENT                             |    |    |     |      |     |     |    |       |       |      |      |       |       |       |       |      |    |      |       |       |      |       |       |       |       |       |       |   |
| NC                                     | 37 | 40 | 40  | 50   | 40  | 34  | 40 | 63.35 | 43.97 | 40   | 42   | 44.17 | 40.54 | 60.66 | 40.54 | 50   | 40 | 50   | 50    | 50    | 19.1 | 29.84 | 20.92 | 40.17 | 29.84 | 29.84 |       |   |
| NG                                     | 35 | 33 | 33  | 33.1 | 33  | 39  | 40 | 25.09 | 34.42 | 26.1 | 28.1 | 33.43 | 37.85 | 29.0  | 37.85 | 34.8 | 40 | 30.6 | 34.8  | 34.82 | 18.6 | 7.36  | 16.73 | 41.43 | 7.86  | 7.86  |       |   |
| DEP                                    | 5  | —  | 9.9 | —    | —   | —   | —  | 11.56 | 5.59  | —    | —    | 8.36  | 5.59  | —     | —     | —    | —  | —    | —     | —     | —    | —     | —     | —     | —     | —     | —     |   |
| DBS                                    | —  | —  | —   | —    | —   | —   | —  | —     | —     | —    | —    | —     | —     | —     | —     | —    | —  | —    | —     | —     | —    | —     | —     | —     | —     | —     | —     |   |
| EC                                     | —  | —  | —   | —    | —   | —   | —  | —     | —     | —    | —    | —     | —     | —     | —     | —    | —  | —    | —     | —     | —    | —     | —     | —     | —     | —     | —     |   |
| 2-NDPA                                 | 2  | 2  | 2   | 2    | 2   | —   | —  | —     | —     | 2    | 2    | —     | —     | —     | —     | —    | —  | —    | —     | —     | —    | —     | —     | —     | —     | —     | 7.5   |   |
| Pb2EH                                  | —  | —  | —   | —    | —   | —   | —  | —     | —     | —    | —    | —     | —     | —     | —     | —    | —  | 2    | 2     | 2     | 2    | —     | —     | —     | —     | —     | —     |   |
| Pbsal                                  | —  | —  | —   | —    | —   | —   | —  | —     | —     | —    | —    | —     | —     | —     | —     | —    | —  | 1.2  | 1.2   | 1.2   | 1.2  | —     | —     | —     | —     | —     | —     |   |
| CW                                     | —  | —  | —   | —    | —   | —   | —  | —     | —     | —    | —    | —     | —     | —     | —     | —    | —  | 1.2  | 1.2   | 1.2   | 1.2  | —     | —     | —     | —     | —     | —     |   |
| 1-B-5-BAT                              | —  | —  | —   | —    | —   | —   | —  | —     | —     | —    | —    | —     | —     | —     | —     | —    | —  | 0.2  | 0.2   | 0.2   | 0.2  | —     | —     | —     | —     | —     | —     |   |
| 5-MAT                                  | —  | 25 | —   | —    | —   | —   | —  | —     | —     | —    | —    | —     | —     | —     | —     | —    | —  | 10.8 | 20    | —     | —    | —     | —     | —     | —     | —     | —     |   |
| 5-EAT                                  | —  | —  | —   | —    | —   | —   | —  | —     | —     | —    | —    | —     | —     | —     | —     | —    | —  | —    | —     | —     | —    | —     | —     | —     | —     | —     | —     |   |
| 5-OAT                                  | —  | —  | —   | —    | —   | —   | —  | —     | —     | —    | —    | —     | —     | —     | —     | —    | —  | 27.9 | —     | —     | —    | —     | —     | —     | —     | —     | —     |   |
| 5-DAT                                  | —  | —  | —   | —    | —   | —   | —  | —     | —     | —    | —    | —     | —     | —     | —     | —    | —  | —    | 16.02 | —     | —    | —     | —     | —     | —     | —     | —     |   |
| 1-M-5-AT                               | 20 | —  | —   | —    | 125 | 125 | —  | —     | —     | —    | —    | —     | —     | —     | —     | —    | —  | —    | —     | 31.9  | —    | —     | —     | —     | —     | —     | —     | — |
| 1-E-5-AT                               | —  | —  | —   | —    | —   | —   | —  | —     | —     | —    | —    | —     | —     | —     | —     | —    | —  | —    | —     | 14.04 | —    | —     | —     | —     | —     | —     | —     | — |
| 2-M-5-AT                               | —  | 25 | 5   | —    | —   | —   | —  | —     | —     | —    | —    | —     | —     | —     | —     | —    | —  | —    | 16.02 | —     | —    | —     | —     | —     | —     | —     | —     |   |
| 1-M-5-MAT                              | —  | —  | —   | —    | —   | —   | —  | —     | —     | —    | —    | —     | —     | —     | —     | —    | —  | 20   | —     | —     | —    | —     | —     | —     | —     | —     | —     |   |
| 1-E-5-EAT                              | —  | —  | —   | —    | —   | —   | —  | —     | —     | —    | —    | —     | —     | —     | —     | —    | —  | —    | —     | —     | —    | —     | —     | —     | —     | —     | —     |   |
| 1-A-4-AAT                              | —  | —  | —   | —    | —   | —   | —  | —     | —     | —    | —    | —     | —     | —     | —     | —    | —  | —    | —     | —     | 10.8 | —     | —     | —     | —     | —     | —     | — |
| 1,5-DMT                                | —  | —  | —   | —    | —   | —   | —  | —     | —     | —    | —    | —     | —     | —     | —     | —    | —  | —    | —     | —     | —    | —     | —     | —     | —     | —     | —     |   |
| E(1-T)A                                | —  | —  | —   | —    | —   | —   | —  | —     | —     | —    | —    | —     | —     | —     | —     | —    | —  | —    | —     | —     | 15.0 | —     | —     | —     | —     | —     | —     | — |
| NO <sub>2</sub> G                      | —  | —  | —   | —    | —   | —   | —  | —     | —     | —    | —    | —     | —     | —     | —     | —    | —  | —    | —     | —     | —    | 54.8  | 54.8  | 51.0  | —     | 54.8  | —     | — |
| 1-(6-T)-2-NO <sub>2</sub> G            | —  | —  | —   | —    | —   | —   | —  | —     | —     | —    | —    | —     | —     | —     | —     | —    | —  | —    | —     | —     | —    | —     | —     | —     | —     | —     | 64.80 |   |
| G, salt of 1-(5-T)-2-NO <sub>2</sub> G | —  | —  | —   | —    | —   | —   | —  | —     | —     | —    | —    | —     | —     | —     | —     | —    | —  | —    | —     | —     | —    | —     | —     | —     | —     | —     | 54.80 |   |

<sup>1</sup> Passed through 200 on 270 mesh.

Key to Table I:

|                                        |                                                            |
|----------------------------------------|------------------------------------------------------------|
| NC                                     | Nitrocellulose (12.6%)                                     |
| NG                                     | Nitroglycerin                                              |
| DEP                                    | Diethyl phthalate                                          |
| DBS                                    | Distyryl sebacate                                          |
| EC                                     | Ethyl centralite                                           |
| 2-NDPA                                 | 2-nitrodiphenylamine                                       |
| Pb2EH                                  | Lead 2-ethylhexoate                                        |
| Pbsal                                  | Lead salicylate                                            |
| CW                                     | Candelilla wax                                             |
| 1-B-5-BAT                              | 1-butyl-5-butylaminotetrazole                              |
| 5-MAT                                  | 5-methylaminotetrazole                                     |
| 5-EAT                                  | 5-ethylaminotetrazole                                      |
| 5-OAT                                  | 5-octylaminotetrazole                                      |
| 5-DAT                                  | 5-decylaminotetrazole                                      |
| 1-M-5-AT                               | 1-methyl-5-aminotetrazole                                  |
| 1-E-5-AT                               | 1-ethyl-5-aminotetrazole                                   |
| 2-M-5-AT                               | 2-methyl-5-aminotetrazole                                  |
| 1-M-5-MAT                              | 1-methyl-5-methylaminotetrazole                            |
| 1-E-5-BAT                              | 1-ethyl-5-ethylaminotetrazole                              |
| 1-A-5-AAT                              | 1-allyl-5-allylaminotetrazole                              |
| 1,5-DMT                                | 1,5-dimethyltetrazole                                      |
| E(1-T)A                                | Ethyl (1-tetrazolyl)acetate                                |
| NO <sub>2</sub> G                      | Nitroguanidine                                             |
| 1-(6-T)-2-NO <sub>2</sub> G            | 1-(6-T)-2-NO <sub>2</sub> G                                |
| G, salt of 1-(5-T)-2-NO <sub>2</sub> G | 1-(5-T)-2-N-(1-(5-tetrazolyl)-2-nitroguanidine)guanidinium |

The tetrazole plasticizers were found to be compatible with the propellant compositions over wide percentage ranges. All of the compositions were well plasticized. Compatibility tests, heat stability and other surveillance tests, flex tests, temperature of explosion tests, second order transitions tests, burning rate tests, and other tests showed that the compositions were satisfactorily plasticized, that they had good surveillance characteristics, had no deleterious effects on required ballistic characteristics of propellants and even increased the burning rate of double base and cool gun propellant compositions.

Typical results of tests performed on representative compositions shown in Table I are included in the following paragraphs.

2-ethyltetrazole and 1,5-dimethyltetrazole were tested as plasticizers for nitrocellulose by the sorption method with the following results: The weight of nitrocellulose in the presence of 2-ethyltetrazole was increased by 182% after 3 hours at 40° C., indicating that this tetrazole solvates nitrocellulose strongly. The weight of nitrocellulose in the presence of 1,5-dimethyltetrazole was increased 45.5% after 75 minutes at 40° C. indicating satisfactory compatibility. 1-ethyl-5-ethylaminotetrazole was found to be compatible with cellulose acetate up to about the 30% level indicating the versatility of the tetrazoles as plasticizers.

50 The finished product in the above cases was highly plasticized and flexible, and the plasticizer was uniformly and homogeneously blended in the nitro cellulose.

The following flex tests performed on compositions of nitrocellulose and representative tetrazoles are included.

55 The tests were made by folding the product back on itself and counting the number of folds before breaking. The tests were performed at 25.5° C.

| Plasticizer                     | Average film thickness, inches | Average Number of folds to break |
|---------------------------------|--------------------------------|----------------------------------|
| None                            | 0.00175                        | 344                              |
| 1-ethyl-5-ethylaminotetrazole   | 0.00177                        | 380                              |
| 1-methyl-5-ethylaminotetrazole  | 0.00207                        | 292                              |
| 1-allyl-5-allylaminotetrazole   | 0.00196                        | 454                              |
| 1-methyl-5-methylaminotetrazole | 0.00177                        | 511                              |

70 Comparison of the results obtained from the plasticized compositions with that obtained on the blank graphically illustrates the general effectiveness of the tetrazole plasticizers.

Second order transition temperatures for representative members from Table I are included below.

| Example No. | Results                                                                                                             |
|-------------|---------------------------------------------------------------------------------------------------------------------|
| 7-----      | No peak in the dielectric power loss curve occurred from -50 to -14° C. Films were tough and flexible.              |
| 16-----     | Peaked at -8° C.                                                                                                    |
| 17-----     | Peaked at -20° C.                                                                                                   |
| 18-----     | Peaked at -18° C. The film was tough and flexible at room temperature.                                              |
| 20-----     | No peak in dielectric power loss curve from -63° C. to -10° C. The film was tough and flexible at room temperature. |
| 24-----     | Peaked at -21° C. Films were tough and flexible.                                                                    |

The above results illustrate the effectiveness of the plasticizers at lower temperatures.

Representative results of conventional temperature of explosion tests for typical compositions of Table I are as follows:

TABLE II

[Average time in seconds for explosion at temperatures shown]

| Example | 298° C. | 330° C. | 372° C. | 397° C. | 412° C. | 428° C. | 458° C. | 485° C. | 510° C. |
|---------|---------|---------|---------|---------|---------|---------|---------|---------|---------|
| 7-----  |         |         | 3.76    |         | 1.80    |         | 1.40    | 1.49    | 1.41    |
| 8-----  |         |         | 2.76    |         | 1.78    |         | 1.27    | 1.19    | 1.33    |
| 9-----  |         |         | 2.43    |         | 1.48    |         | 1.13    | 1.18    | 1.03    |
| 12----- |         |         | 2.03    | 1.28    |         | 0.94    | 0.72    | 0.83    | -----   |

The extended time of explosion at the temperatures shown further indicates the stability of the compositions.

To supplement the heat stability tests given below for double base propellant formulations incorporating the plasticizers, heat stability test results obtained on Examples 22 and 25, cool gun propellant compositions, are included as follows: The compositions darkened in heat stability tests at 136° C. but did not explode during 8 hours. Oxides of nitrogen were not evolved, as indicated by the fact that the methyl violet paper used for indicating stability did not develop a pink or salmon color.

Graphs of representative results of standard burning rate tests performed on typical compositions of Table I are included as FIGS. 1, 2, 3 and 4. The graphs are logarithmic plots in which the burning rate of the propellant is plotted against pressure, the divisions on the abscissa representing multiples of 100. Inspection of the graphs shows that ballistic properties of the propellants are actually enhanced by incorporation of the plasticizers therein. For example, comparison of the graphs for the blanks 8 and 14 of FIG. 2 and the blank 21 of FIG.

4 with the graphs for the other compositions shows that the burning rate is appreciably increased by the presence of the plasticizer. While some of this effect for Examples 25, 26 and 27 of FIG. 4 must be attributed to the use of the new cool gun base compounds, it is quite obvious that some of the effect is due to the plasticizers.

Tables III and IV below present results of heat stability tests performed on propellant compositions containing varying amounts of tetrazole plasticizers. For making the tests the weighed ingredients were dissolved in acetone by tumbling in sealed bottles for 24 hours and the resulting solutions cast into films on glass and dried for 2.5 days.

TABLE III

15 [The compositions consisted of 37% nitrocellulose (12.6% N), 30% nitroglycerin, and 33% of the tetrazole derivative—tests performed at 136° C.]

| Example | Compound      | First salmon color on methyl violet paper, min. | Definite salmon color, min. | Explosion or decomposition min. |
|---------|---------------|-------------------------------------------------|-----------------------------|---------------------------------|
| 20----- | 1,5-DMT       | -----                                           | 13                          | 53-56                           |
| 28----- | 5-MAT         | 25                                              | 39-42                       | -----                           |
| 29----- | 5-DMAT        | 3                                               | 8-16                        | -----                           |
| 30----- | 5-DAAT        | -----                                           | 8-10                        | -----                           |
| 31----- | 5-EAT         | 16                                              | 26                          | 32                              |
| 32----- | 5-HAT         | 32                                              | -----                       | 33                              |
| 33----- | 5-PAT         | 7                                               | 11                          | 135                             |
| 34----- | 1-M-5-AT      | 5                                               | -----                       | 10-13                           |
| 35----- | 1-E-5-AT      | -----                                           | 9                           | -----                           |
| 36----- | 1-(m-CP)-5-AT | 28                                              | -----                       | 150-180                         |
| 37----- | 2-M-5-AT      | 25                                              | -----                       | 28-29                           |
| 38----- | 2-E-5-AT      | 21                                              | -----                       | 29-30                           |
| 39----- | 1-M-5-MAT     | 30                                              | 60                          | (1)                             |
| 40----- | 1-A-6-AAT     | -----                                           | -----                       | (2)                             |
| 41----- | 2-M-5-MAT     | 117                                             | 210                         | (1)                             |
| 42----- | 2-M-5-NT      | 11                                              | 13                          | 35                              |
| 43----- | 2-M-5-DMAT    | (3)                                             | 25                          | -----                           |
| 44----- | 1-M-5-DMAT    | -----                                           | -----                       | -----                           |

35 <sup>1</sup> Melted but no explosion.

<sup>2</sup> Melted after 10 minutes, frothed after 55 minutes.

<sup>3</sup> Melted after 7 minutes, frothed after 20 minutes.

Key to Table III excluding those terms used in Table I:

5-DMAT—5-dimethylaminotetrazole

5-DAAT—5-diallylaminotetrazole

5-HAT—5-heptylaminotetrazole

5-PAT—5-phenylaminotetrazole

1-(m-CP)-5-AT—1-(m-chlorophenyl)-5-aminotetrazole

2-E-5-AT—2-ethyl-5-aminotetrazole

2-M-5-MAT—2-methyl-1-5-methylaminotetrazole

2-M-5-NT—2-methyl-5-nitrotetrazole

1-M-5-DMAT—1-methyl-5-dimethylaminotetrazole

40 In order to illustrate the heat stability of different percentage compositions of propellants as well as the compatibility of the tetrazole plasticizers with a conventional stabilizer, 2-nitrodiphenylamine, the results of Table IV are included.

TABLE IV

| Example                                            | 45   | 46    | 47   | 48   | 49    | 50   | 51   | 52    | 53    | 54    | 55   | 56    | 57    | 58   |
|----------------------------------------------------|------|-------|------|------|-------|------|------|-------|-------|-------|------|-------|-------|------|
| Ingredient:                                        |      |       |      |      |       |      |      |       |       |       |      |       |       |      |
| NC (12.6%)                                         | 37   | 46    | 32   | 46   | 37    | 46   | 37   | 37    | 54.8  | 50    | 40   | 40    | 40    | 51   |
| NG                                                 | 28.5 | 27    | 26   | 27   | 28.5  | 27   | 28.5 | 28.5  | 42.3  | 36    | 36   | 36    | 36    | 25   |
| 2-NDPA                                             | 2    | 2     | 2    | 2    | 2     | 2    | 2    | 2     | 2.9   | 2     | 2    | 2     | 2     | 2    |
| DEP                                                | 2.5  |       | 5    |      | 2.5   |      |      |       |       | 50    |      |       |       | 22   |
| Tetrazole:                                         |      |       | 35   |      |       |      |      |       |       |       |      |       |       |      |
| 1,5-DMT                                            |      |       |      |      |       |      |      |       |       |       |      |       |       |      |
| 5-MAT                                              | 30   |       |      |      |       |      |      |       |       |       |      |       |       |      |
| 5-EAT                                              |      |       |      |      |       |      |      |       |       |       |      |       |       |      |
| 5-DMAT                                             |      |       |      |      |       |      |      |       |       |       |      |       |       |      |
| 5-DAAT                                             |      |       |      |      |       |      |      |       |       |       |      |       |       |      |
| 1-M-5-AT                                           |      |       |      |      |       |      |      |       |       |       |      |       |       |      |
| 1-E-5-AT                                           |      |       |      |      |       |      |      |       |       |       |      |       |       |      |
| 1-M-5-MAT                                          |      | 25    |      |      |       |      |      |       |       |       |      |       |       |      |
| 1-E-5-EAT                                          |      |       |      |      |       |      |      |       |       |       |      |       |       |      |
| 2-M-5-AT                                           |      |       |      |      |       |      |      |       |       |       |      |       |       |      |
| 2-M-5-MAT                                          |      |       |      |      |       |      |      |       |       |       |      |       |       |      |
| Heat stability, 106° C.:                           |      |       |      |      |       |      |      |       |       |       |      |       |       |      |
| First salmon color on methyl violet paper, minutes | None | 270   | 43   | None | 47    | None |      |       |       |       | 107  | 110   |       |      |
| Definite salmon color, minutes                     | None |       | 53   | None |       | None |      |       |       |       |      |       |       |      |
| Explosion or extensive decomposition, minutes.     | None | None  | None | None | None  | None |      |       |       |       | None | None  | None  |      |
| Heat stability, 136° C.:                           |      |       |      |      |       |      |      |       |       |       |      |       |       |      |
| First salmon color, minutes                        | 27   | 27-46 |      | 53   | 28    |      | 38   | 28-38 | 14-35 | 9-17  |      | 7.9   | 10-15 | 10   |
| Definite salmon color, minutes                     |      | 35    |      | 71   | 44    |      |      |       | 16-42 | 11-22 |      | 10    | 16    | 50   |
| Explosion or extensive decomposition, minutes.     | 64   | None  | 12   | None | 40-49 | 9.5  | 58   | None  | 135   | 28-33 | 7    | 43-68 | 52    | None |

As is illustrated by the examples in Tables I, III and IV the tetrazole plasticizing agents are effective within a range of 5 to 50 percent by weight of the compositions.

Numerous tests performed on 5-aminotetrazole showed that it was not the equivalent of the other tetrazoles as a plasticizer. For example, it showed no compatibility with either double base or cool gun propellants, and did not have any plasticizing effect on these propellants. This compound forms a heterogeneous rather than a homogeneous system with the propellant, and as a result the composite propellant formulation has poorer physical properties than the homogeneous system formed by this invention. Further, the fact that this compound is hygroscopic seriously detracts from its value as a component of propellant formulations. As respects solvating and plasticizing power this compound is not the equivalent of the tetrazole plasticizers set forth above.

A number of the tetrazole derivatives and the cool gun propellants disclosed above are new or relatively unknown, so that it is believed expedient to cite references to methods of preparation for those which have been previously prepared and to give the method of preparation for those which are new. The method of preparation of the following compounds is given in "Preparation and Isomerization of 5-Alkylaminotetrazoles," by William G. Finnegan, Ronald A. Henry, and Eugene Lieber, published in volume 18, No. 7, of The Journal of Organic Chemistry, July 1953: 5-methylaminotetrazole, 5-dimethylaminotetrazole, 5-ethylaminotetrazole, 5-phenylaminotetrazole, 1-methyl-5-aminotetrazole, 1-ethyl-5-aminotetrazole, 1-methyl-5-methylaminotetrazole, 1-methyl-5-dimethylaminotetrazole and 1-ethyl-5-ethylaminotetrazole. Methods of preparing the following compounds are found in the article. "Preparation and Hydrogenation of Azomethines Derived From 5-Aminotetrazole," by Ronald A. Henry and William G. Finnegan, published in The Journal of the American Chemical Society, 76, 926 (1954): 5-heptylaminotetrazole, 5-octylaminotetrazole and 5-decylaminotetrazole. The preparation of 1-(m-chlorophenyl)-5-aminotetrazole is given in the article "Thermal Isomerization of Substituted 5-Aminotetrazoles," by Ronald A. Henry, William G. Finnegan, and Eugene Lieber, published in The Journal of the American Chemical Society, 76, 88 (1954). The method of preparing the following compounds is given in the article, "Mono-Alkylation of Sodium 5-Aminotetrazole in Aqueous Medium," by Ronald A. Henry and William G. Finnegan, published in The Journal of the American Chemical Society, 76, 923 (1954): 2-methyl-5-aminotetrazole, 2-ethyl-5-aminotetrazole, 2-methyl-5-methylaminotetrazole and 2-methyl-5-nitrotetrazole. The methods for preparing tetrazole, 5-dimethyltetrazole, 5-diallylaminotetrazole and 2-ethyltetrazole are well known in the art. The following are new compounds for which the methods of preparation are given below: 1-butyl-5-butylaminotetrazole, 1-allyl-5-allylaminotetrazole, ethyl (1-tetrazolyl)acetate, ethyl (2-tetrazolyl)acetate,  $\beta$ -(1-tetrazolyl)ethyl acetate,  $\beta$ -(2-tetrazolyl)ethyl acetate, ethyl (1-methyl-5-tetrazolyl)acetate, ethyl (2-methyl-5-tetrazolyl)acetate, 1,4-bis (1-methyl-5-tetrazolyl)butane, 1,4-bis (2-methyl-5-tetrazolyl)butane, 1-(5-tetrazolyl)-2-nitroguanidine and the guanidinium salt of 1-(5-tetrazolyl)-2-nitroguanidine.

#### 1-*Allyl*-5-*Allylaminotetrazole*

The compound was prepared in 82% yield from 1,3-diallylthiourea by the method of Finnegan, Henry, and Lieber. (Journal of Organic Chemistry, 18, 779 (1953).) After three recrystallizations from diethyl ether, the melting point of the product was found to be 48.5-49.5° C.

| Analysis                                                    | Carbon | Hydrogen | Nitrogen |
|-------------------------------------------------------------|--------|----------|----------|
| Calculated (C <sub>7</sub> H <sub>11</sub> N <sub>5</sub> ) | 51.44  | 6.69     | 41.89    |
| Found                                                       | 51.08  | 6.31     | 42.63    |

#### 1-*Butyl*-5-*Butylaminotetrazole*

The compound was made in a similar fashion from 1,3-dibutylthiourea with a yield of 86%. Two recrystallizations from ethyl acetate-petroleum ether (1:10) gave a product melting between 74-76° C.

| Analysis                                                    | Carbon      | Hydrogen  | Nitrogen |
|-------------------------------------------------------------|-------------|-----------|----------|
| Calculated (C <sub>9</sub> H <sub>19</sub> N <sub>5</sub> ) | 54.79       | 9.71      | 35.51    |
| Found                                                       | 54.92-54.86 | 9.22-9.23 | 35.66    |

#### Ethyl (1- and 2-Tetrazolyl)Acetates

Tetrazole (41.9 g., 0.599 mole) was suspended in 100 ml. of absolute ethanol in a one liter, three necked, round bottom flask, equipped with a mechanical stirrer, additional funnel, and a reflux condensed. The tetrazole was neutralized to the phenolphthalein end point by the addition of a solution of 39.6 g. (0.599 mole) of 85% potassium hydroxide in 100 ml. of 95% ethanol, and the solution was heated to boiling on a steam bath. Ethyl bromoacetate (100 g., 0.599 mole) was then added as rapidly as the reflux permitted and the resulting homogeneous solution was heated and stirred for two hours. Potassium bromide precipitated as the reaction proceeded. The reaction mixture was then cooled to room temperature, the potassium bromide removed by filtration and the filtrate evaporated to dryness in vacuo on a steam bath. The residue was extracted with three 100 ml. portions of methylene chloride. The methylene chloride solution was dried over magnesium sulfate and evaporated to dryness, leaving 86.2 g. (92.2% yield) of impure ethyl tetrazolyl-acetates as a viscous oil. Distillation at 1 mm. pressure yielded 23.2 g. (24.8% yield) of ethyl (2-tetrazolyl)-acetate, B.P. 83.5-84° C., M.P. 51-52° C.

| Analysis                                                                  | Carbon | Hydrogen | Nitrogen |
|---------------------------------------------------------------------------|--------|----------|----------|
| Calculated (C <sub>5</sub> H <sub>8</sub> O <sub>2</sub> N <sub>4</sub> ) | 38.46  | 5.16     | 35.89    |
| Found                                                                     | 38.10  | 4.50     | 35.71    |

The residue of ethyl (1-tetrazolyl)acetate (42.1 g., yield—45%) was distilled in a Hickman still at 10<sup>-4</sup> mm. pressure and 90-100° C. pot temperature.

| Analysis                                                                  | Carbon | Hydrogen | Nitrogen |
|---------------------------------------------------------------------------|--------|----------|----------|
| Calculated (C <sub>5</sub> H <sub>8</sub> O <sub>2</sub> N <sub>4</sub> ) | 38.46  | 5.16     | 35.89    |
| Found                                                                     | 38.99  | 4.69     | 35.06    |

#### $\beta$ -(1- and 2-Tetrazolyl)Ethyl Acetates

The compounds were prepared from 1- and 2-(2-hydroxyethyl)tetrazoles which were prepared as follows: A suspension of 70 g. (1.0 mole) of recrystallized tetrazole in 150 ml. of water in a two liter round bottom flask was neutralized to the phenolphthalein end point with a solution of 41.25 g. (1.0 mole) of 97% sodium hydroxide in 150 ml. of water. A reflux condenser was attached to the flask and the solution was heated to reflux. 2-chloroethanol (101 g., 1.25 moles) was then added through the condenser as rapidly as the rate of reflux permitted. After the solution had been refluxed overnight, the water was removed by vacuum evaporation on a steam bath. The hydroxyethyltetrazoles in the residue were separated from the sodium chloride by extraction with one 300 ml. and three 100 ml. portions of boiling acetone. The acetone solution was vacuum evaporated to leave 113.3 g. (99.34%) of mixed hydroxyethyltetrazoles. This mixture was dehydrated by azeotropic distillation with benzene and the excess benzene removed by vacuum evaporation. Acetylation of the hydroxyethyltetrazoles was accomplished by heating the mixture with a large excess of acetic anhydride for 2 hours on a steam bath. The excess anhydride and the acetic acid produced were removed by vacuum distillation. Fractionations of the residue

yielded 43.6 g. (27.94% based on tetrazole) of  $\beta$ -(2-tetrazolyl)ethyl acetate, B.P. 81-84° C. at ca. 1 mm., and 47.6 g. (30.5% yield) of  $\beta$ -(1-tetrazolyl)ethyl acetate which was distilled in a Hickman still at 10<sup>-4</sup> mm. pressure and 95° C. pot temperature.

| Analysis                                                                                                                  | Carbon | Hydrogen | Nitrogen |
|---------------------------------------------------------------------------------------------------------------------------|--------|----------|----------|
| $\beta$ -(2-tetrazolyl) ethyl acetate:<br>Calculated (C <sub>8</sub> H <sub>10</sub> O <sub>2</sub> N <sub>4</sub> )----- | 38.46  | 5.16     | 35.89    |
| Found-----                                                                                                                | 37.74  | 3.93     | 37.71    |
| $\beta$ -(1-tetrazolyl) ethyl acetate:<br>Calculated (C <sub>8</sub> H <sub>10</sub> O <sub>2</sub> N <sub>4</sub> )----- | 38.46  | 5.16     | 35.89    |
| Found-----                                                                                                                | 40.46  | 3.29     | 33.21    |

#### Ethyl (1- and 2-Methyl-5-Tetrazolyl) Acetates

The compounds were made from ethyl (5-tetrazolyl) acetate. Ethyl (5-tetrazolyl) acetate was synthesized from ethyl cyanoacetate by the alternate procedure of Mihina and Herbst (Journal of Organic Chemistry, vol. 15, 1082 (1950)). A one mole scale reaction yielded 52.5 g. (33.7%) ethyl (5-tetrazolyl) acetate; 14.0 g. (12.4%) of ethyl cyanoacetate and 21.2 g. of (24.9%) of cyanoacetic acid were recovered.

| Analysis                                                                        | Carbon | Hydrogen | Nitrogen |
|---------------------------------------------------------------------------------|--------|----------|----------|
| Calculated (C <sub>8</sub> H <sub>10</sub> O <sub>2</sub> N <sub>4</sub> )----- | 38.46  | 5.16     | 35.89    |
| Found-----                                                                      | 38.30  | 4.46     | 35.88    |

For the preparation of ethyl (1- and 2-methyl-5-tetrazolyl)-acetates, ethyl-(5-tetrazolyl) acetate (62.4 g., 0.4 mole) in 200 ml. of 95% ethanol was neutralized to a phenolphthalein end point with a 50 percent solution of sodium hydroxide. The solution contained in the two liter round bottom flask equipped with a condenser was then heated to reflux and 62.5 g. (0.44 mole) of methyl iodide was added through the condenser as fast as the rate of reflux permitted. After a total of 17 hours reflux, the solution was stripped to dryness in vacuo on a steam bath and the residue extracted with three 100 ml. portions of methylene chloride. The methylene chloride solution was dried over magnesium sulfate, filtered and evaporated. The residue from the methylene chloride solution was dissolved in 200 ml. of isopropanol. Chilling this solution yielded 20.53 g. (30.2%) of ethyl (1-methyl-5-tetrazolyl) acetate having a melting point of 67-68° C.

| Analysis                                                                        | Carbon | Hydrogen | Nitrogen |
|---------------------------------------------------------------------------------|--------|----------|----------|
| Calculated (C <sub>8</sub> H <sub>10</sub> O <sub>2</sub> N <sub>4</sub> )----- | 42.35  | 5.92     | 32.93    |
| Found-----                                                                      | 41.41  | 5.80     | 32.27    |

The isopropanol filtrate was evaporated to dryness and the residue was distilled, yielding 28.95 g. (42.6% yield) of ethyl (2-methyl-5-tetrazolyl)acetate having a boiling point of 103°-104° C. at 0.8 mm. pressure.

| Analysis                                                                        | Carbon | Hydrogen | Nitrogen |
|---------------------------------------------------------------------------------|--------|----------|----------|
| Calculated (C <sub>8</sub> H <sub>10</sub> O <sub>2</sub> N <sub>4</sub> )----- | 42.35  | 5.92     | 32.93    |
| Found-----                                                                      | 41.79  | 5.35     | 33.27    |

Recrystallization of the distillation residue yielded an additional 7.13 g. (10.5%) of ethyl (1-methyl-5-tetrazolyl) acetate.

#### 1,4-Bis (1- and 2-methyl-5-Tetrazolyl)Butanes

The compounds were made from 1,4-bis (5-tetrazolyl)-butane. 1,4-bis (5-tetrazolyl)butane was prepared in 80.5% yield by reacting 11.2 g. (0.1037 mole) of adiponitrile, 14.0 g. (0.215 mole) of sodium azide in 17.0 ml. of glacial acetic acid and 25 ml. of absolute ethanol at 150° C. for 96 hours in a 180 ml. capacity high pressure reactor following the procedure of J. S. Mihina and R. M.

Herbert (Journal of Organic Chemistry, vol. 15, 1082 (1950)). The product was isolated by dissolving the reaction mixture in 100 ml. of ice water and acidifying the solution with 20 ml. of concentrated hydrochloric acid. 5 The precipitated 1,4-bis (5-tetrazolyl)butane was removed by filtration, washed on the filter with three, 50 ml. portions of ice water and air dried to give 16.18 g. of product. Recrystallization from water yielded 14.04 g. of pure product having a melting point of 204-205° C.

| Analysis                                                          | Carbon | Hydrogen | Nitrogen |
|-------------------------------------------------------------------|--------|----------|----------|
| Calculated (C <sub>10</sub> H <sub>16</sub> N <sub>8</sub> )----- | 37.10  | 5.19     | 56.71    |
| Found-----                                                        | 37.15  | 4.83     | 58.12    |

10 For the preparation of the 1,4-bis (1- and 2-methyl-5-tetrazolyl)butanes, 1,4-bis (5-tetrazolyl)butane (12.19 g., 0.063 mole) was suspended in 50 ml. of water, neutralized to a phenolphthalein end-point with 50% sodium hydroxide solution and the solution diluted to a total volume of 100 ml. After the solution was warmed to 70° C., 17.5 g. (0.1386 mole) of dimethyl sulfate was added dropwise with stirring; 50% sodium hydroxide was added as necessary to maintain the phenolphthalein endpoint. The 20 addition of dimethyl sulfate was complete in 30 minutes and the solution was stirred at 70° C. for an additional two hours. The solution was then concentrated in vacuo on a steam bath to about 25 ml. and extracted with three 50 ml. portions of ethylene chloride. The ethylene chloride solution was evaporated to dryness leaving 10.18 g. (72.8%) of methylated products as a semi-solid residue. This residue was slurried with 100 ml. of cold acetone and 2.03 g. (14.5%) of solid having a melting point of 139-140° C. were removed by filtration. Recrystallization 30 from ethanol did not raise the melting point.

Analysis: Nitrogen  
Calculated (C<sub>8</sub>H<sub>14</sub>N<sub>8</sub>)----- 50.43  
Found ----- 50.40-50.25

40 This material was probably 1,4-bis (1-methyl-5-tetrazolyl)butane. The acetone filtrate was evaporated to dryness, leaving 7.98 g. (52.0%) of soft solid which was probably a mixture of 1,4-bis (2-methyl-5-tetrazolyl)-butane and 1-(1-methyl-5-tetrazolyl)-4-(2-methyl-5-tetrazolyl)butane.

45 Analysis: Nitrogen  
Calculated (C<sub>8</sub>H<sub>14</sub>N<sub>8</sub>)----- 50.43  
Found ----- 51.61-51.13-51.5

50 The basic solution remaining after extraction of the methylated bis tetrazolyl butanes was acidified with concentrated hydrochloric acid and extracted with ethylene chloride. Evaporation of the ethylene chloride left 2.92 g. of partially methylated products and starting material.

#### 1-(5-Tetrazolyl)-2-Nitroguanidine

A solution of 6.1 g. (0.072 mole) of anhydrous 5-amino-tetrazole in 150 ml. of water was adjusted to the phenolphthalein endpoint with a 50% solution of sodium hydroxide. S-methyl-N-nitrosothiourea (9.6 g., 0.072 mole) was then added and the resulting solution was heated under reflux on a steam bath for 12 hours. The evolution of methyl mercaptan began immediately and was essentially complete at the end of the heating period. The solution was cooled, filtered from a small amount of insoluble material, adjusted to pH 2 with concentrated hydrochloric acid, and cooled overnight at 5° C. The product was removed by filtration, washed with two small volumes of cold water, and air dried. The yield was 6.35 g. (51.6%). From the aqueous mother liquors 1.5 g. (anhydrous) of unreacted 5-aminotetrazole was recovered. (In a second experiment the yield was 37.8%.) The crude product was recrystallized once from water (about 10 ml./g.) to give a fine white granular powder which 70 did not melt below 250° C. when heated slowly, but which 75

decomposed vigorously at 240-245° C. when plunged into a hot bath at this temperature.

| Analysis                                                                                  | Carbon | Hydrogen | Nitrogen |
|-------------------------------------------------------------------------------------------|--------|----------|----------|
| Calculated (C <sub>2</sub> H <sub>4</sub> N <sub>4</sub> O <sub>2</sub> H <sub>2</sub> O) | 12.63  | 3.18     | 58.94    |
| Found                                                                                     | 13.56  | 3.27     | 58.0     |
| Calculated (C <sub>2</sub> H <sub>4</sub> N <sub>8</sub> O <sub>2</sub> )                 | 13.96  | 2.34     | 65.11    |
| Found                                                                                     | 14.1   | 2.14     | 65.5     |

*Guanidinium Salt of 1-(5-Tetrazolyl)-2-Nitroguanidine*

A slurry of 17.0 g. of anhydrous 5-aminotetrazole in 80 ml. of cold water was treated with 18.0 g. of guanidinium carbonate at such a rate that the evolution of carbon dioxide was not excessive. When complete solution of these reactants was attained, 120 ml. of 95% ethanol and 29.4 g. of 1-methyl-1-nitroso-2-nitroguanidine were added. A slow evolution of gas began immediately; after one week at room temperature the orange-yellow methylnitrosonitroguanidine had disappeared completely and had been replaced by a white granular solid. The mixture was heated to dissolve the solid phase, then cooled overnight at 5° C. The solid was removed by filtration, washed with a small volume of cold water, and air dried. The yield was 10.3 g. A second crop of 5.0 g. was obtained by evaporating the filtrate under reduced pressure to 100 ml. and recooling to 5° C. The total recovery of guanidinium salt, melting point 236-240° C., amounted to 33.1% of theory. The impure salt can be recrystallized from either water (10 ml./g.) or from 60% ethanol (20 ml./g.) and is recovered as white, rather fluffy rosettes which decompose at 240-242° C. when plunged into a hot bath.

| Analysis                                                                   | Carbon      | Hydrogen  | Nitrogen  |
|----------------------------------------------------------------------------|-------------|-----------|-----------|
| Calculated (C <sub>3</sub> H <sub>6</sub> N <sub>11</sub> O <sub>2</sub> ) | 15.58       | 3.92      | 66.65     |
| Found                                                                      | 15.55-15.73 | 4.03-4.24 | 67.1-64.5 |

The utility of 1-(5-tetrazolyl)-2-nitroguanidine and its guanidinium salt as substitutes for nitroguanidine in cool gun propellants is well demonstrated by the burning rate curves, Examples 26 and 27, respectively, of these two compounds presented in FIG. 4, the increase in burning rate being largely due to the presence of these compounds. Stability tests demonstrated that they have acceptable surveillance characteristics. In general, the use of 1-(5-tetrazolyl)-2-nitroguanidine produces a two to threefold increase in the burning rate over that shown by comparable formulations with nitroguanidine, as shown in FIG. 4. The guanidinium salt of this compound in propellant compositions is seen to increase the burning rate appreciably over comparable formulations containing nitroguanidine.

A distinct advantage of the invention, resulting from the fact that the plasticizing agents contain a large percentage of nitrogen, is the fact that the agents contribute a smaller negative heat of explosion to the formulations, thus resulting in a more efficient propellant in that more nitrocellulose and less nitroglycerin can be used. For example, the conventional plasticizers, diethylphthalate and ethyl centralite have heats of explosion of -1761 and -2412, respectively, while the heats of explosion of 1-ethyl-5-ethylaminotetrazole, ethyl (1-tetrazolyl)acetate and 1,5-dimethyl tetrazole are -1225, -693 and -970.7 cal./gram, respectively.

A further advantage of the invention over the prior art is the fact that it provides homogeneous, single phase, cool propellant compositions.

From the above description it is seen that the invention provides novel and effective propellant compositions, characterized by the addition thereto of tetrazole derivatives, these derivatives serving not only as effective plasticizers for the preparation of homogeneous compo-

sitions but also increasing the burning rate of the compositions without detracting from their surveillance and other requisite characteristics.

Obviously many modifications and variations of the present invention are possible in the light of the above teachings. It is therefore to be understood that within the scope of the appended claims the invention may be practiced otherwise than as specifically described.

What is claimed is:

10. Gas producing compositions consisting essentially of a first component about 45 to about 90% of a material selected from the class consisting of nitrocellulose-nitroglycerin systems in which the components are present in weight percents of about 30-60 and 25-45, respectively; nitrocellulose-nitroglycerin-nitroguanidine systems in which the components are present in weight percents of about 19-30, 7-19 and 51-57.5, respectively; nitrocellulose-nitroglycerin-1-(5-tetrazolyl)-2-nitroguanidine systems in which the components are present in weight percents of about 30, 7 and 55, respectively; and nitrocellulose-nitroglycerin-guanidinium salt of 1-(5-tetrazolyl)-2-nitroguanidine systems in which the components are present in weight percents of about 30, 7 and 55, respectively, and as a second component from about 5 to about 50 weight percent of a material selected from the class consisting of



and



wherein R is hydrogen, lower alkyl, lower alkylene, nitro, lower aminoalkyl, lower aminoalkylene, amino-phenyl, lower carboalkoxyalkyl, and lower acyloxyalkyl; and R<sub>1</sub> and R<sub>2</sub> are hydrogen, lower alkyl, lower alkylene, phenyl, lower carboalkoxy-alkyl and lower acyloxy-alkyl, with the limitation that R<sub>1</sub> and R<sub>2</sub> are not hydrogen when R is hydrogen.

40. The gas producing composition of claim 1 in which said second component is 1-ethyl-5-ethylaminotetrazole.
3. The gas producing composition of claim 1 in which said second component is 1,5-dimethyltetrazole.
4. The gas producing composition of claim 1 in which said second component is 2-methyl-5-methylaminotetrazole.

5. The gas producing composition of claim 1 in which said second component is 2-methyl-5-nitrotetrazole.

6. The gas producing composition of claim 1 in which said second component is ethyl (1-tetrazolyl)acetate.

7. The gas producing composition of claim 1 in which said first component is a nitrocellulose-nitroglycerin-nitroguanidine system and said second component is 1-ethyl-5-ethylaminotetrazole.

60. The gas producing composition of claim 1 in which said first component is a nitrocellulose-nitroglycerin system and said second component is 1-ethyl-5-ethylaminotetrazole.
8. The gas producing composition of claim 1 in which said second component is 1,5-dimethyltetrazole.

9. The gas producing composition of claim 8 in which said second component is 1,5-dimethyltetrazole.
10. The gas producing composition of claim 8 in which said second component is 2-methyl-5-methylaminotetrazole.

11. The gas producing composition of claim 8 in which said second component is ethyl (1-tetrazolyl)acetate.

References Cited in the file of this patent

UNITED STATES PATENTS